

# UNITED STATES PATENT OFFICE.

THOMAS DAVIES NICHOLLS, OF SKEWEN, NEAR NEATH, AND CHRISTOPHER JAMES, OF SWANSEA, ENGLAND.

## METHOD OF REFINING COPPER.

SPECIFICATION forming part of Letters Patent No. 532,809, dated January 22, 1895.

Application filed June 18, 1891, Serial No. 396,715. (No specimens.) Patented in England November 21, 1890, No. 18,898; in Spain July 9, 1891, No. 12,214; in Italy July 14, 1891, XXV, 29,950, LVIII, 450; in Newfoundland August 10, 1891; in France September 30, 1891, No. 214,025, and in Cape of Good Hope February 27, 1892, No. 741.

*To all whom it may concern:*

Be it known that we, THOMAS DAVIES NICHOLLS, residing at Glan-Mor Villas, Skewen, near Neath, and CHRISTOPHER JAMES, of Ida Villa, Swansea, in the county of Glamorgan, England, have invented an Improved Method of Refining Copper, of which the following is a specification.

The invention has been patented in Great Britain, No. 18,898, dated November 21, 1890; in France, No. 214,025, dated September 30, 1891; in Italy, XXV, 29,950, LVIII, 450, dated July 14, 1891; in Spain, No. 12,214, dated July 9, 1891; in Newfoundland August 10, 1891, and in the Colony of the Cape of Good Hope, No. 741, dated February 27, 1892.

This invention relates to an improved method of producing refined copper from copper matte, regulus or precipitate and the operations entailed therein are conducted as follows: In the ordinary methods now in use copper matte or regulus, consisting principally of copper and sulphur, is piled, in as large pieces as practicable, in a "roaster" furnace, and slowly sweated down while exposed to a current of air let in through the side door of the furnace,—through air holes or plugs, or through passages arranged through the fire by the workman; thus burning off the sulphur nearly, and leaving the copper, after melting and skimming to be tapped out as "pimple" or "blister" copper. This operation takes seldom less than twenty four hours for the production of three tons of "pimple" or "blister" copper from matte of seventy-five or seventy-six per cent. while a large amount of copper passes into the roaster slags, which have to be resmelted. The "blister" or "pimple" copper, thus made, is then filled as pigs into a refinery furnace and again sweated down under an oxidizing flame, skimmed, refined and brought to the required pitch, and finally laded into cakes, ingots, anodes, &c.

In the new method proposed herein, we avoid the expensive and wasteful two operations of roasting and melting, first in a "roaster" and again in a "refinery" furnace

by substituting a calcination of a portion only of the matte, then mixing this calcined portion with a suitable portion of raw (uncalcined) matte. This mixture is then charged directly into a "refinery" furnace, and melted at once into impure metallic copper or blister copper containing about ninety-seven and one-half per cent. of copper with sulphur and traces of other metallic impurities which is brittle and un-malleable. It is then refined in the usual way in the hearth of the same refinery furnace in which the calcined and raw matte (of say seventy-six to seventy-eight per cent. of copper) has been smelted. This usual way of refining is by oxidation of the liquid metal in the hearth while it is being "flapped" or stirred by suitable hand hoes or "flaps" until all the sulphur and any traces of iron, nickel, arsenic, and antimony have been oxidized and removed as slag, volatile bodies being volatilized and any excess of oxidation is then removed by "poling" with timber poles. The metal is thus reduced to refined copper of 99.6 or one hundred per cent. of copper by the continuous process in the one furnace and is malleable and of great tenacity, fit for the market, and is then formed as required into cakes, ingots, anodes, &c.

We find in practice that the best and most economical matte for our process is one of about seventy-six to seventy-eight per cent. of copper, matte of this pitch containing but little iron, and so making very little slag in the "refinery" furnace. The whole of this matte is crushed through a three-eighths inch screen (or smaller if convenient though when rich matte is treated fine dust is wasteful). A portion of our matte or regulus we calcine in reverberatory calciners or revolving cylinder calciners or any calciner at present in ordinary use. The calcination of this portion of matte is so conducted until it is "dead" and mixed with such a portion of raw matte as will suffice (when melted together) to render all the copper in both portions as metallic copper of a pitch similar to the "blister" copper from the ordinary "roaster." Both portions, so mixed, form the refinery charge.

The reactions which insure the success of this method of working may be described as follows: Copper matte of the preferred pitch consists essentially of copper sulphide ( $Cu_2S$ ).

- 5 This when calcined perfectly would be changed to copper oxide ( $CuO$ ) of equal weight with the copper sulphide operated on. This copper oxide ( $CuO$ ) upon being melted with its own weight of raw copper matte ( $Cu_2S$ ) 10 produces metallic Cu from both portions with the evolution of nearly all the sulphur and oxygen as sulphur gas, as expressed by the well known formula:



- 15 In practice we find that to perfectly calcine the portion of matte so treated is tedious and expensive, the calcination of the copper sulphide to red oxide of copper ( $Cu_2O$ ) being 20 comparatively easy while the further calcination of this red oxide to black oxide ( $CuO$ ) requires so much longer time and greater heat, that although the black oxide will carry its own weight of raw matte in the refinery 25 charge, it is cheaper to only so far calcine our matte that upon trial it is found that about two parts of calcined matte and one part of raw matte will, upon melting render all the copper as "blister" copper with very little 30 slag.

We claim, that by treating only about two thirds of our matte in a calciner, and then melting the total quantity in a refinery furnace with the immediate production of metallic copper, which is at once refined in the hearth of the same furnace in which the mixed calcined and raw matte has been smelted without remelting, good copper is produced at far less direct cost than by the 40 ordinary roasting and refining processes; that more copper is obtained in a salable form and far less slags produced than by the roasting, melting and skimming, first in a roaster, and again in a refinery furnace with the production of heavy slags in each operation.

In our method of working, we find that all volatile impurities (arsenic, antimony, bismuth, &c.) are more freely got rid of than in the roasting process, partly in the thorough 50 calcination of the calcined portion, and again during the evolution of the large volume of sulphur gas, given off on melting the mixed charge in the refinery, aided by the intense

chemical heat developed by there action set up by the combining of the melting oxide 55 and sulphide.

The non - volatile impurities (iron, nickel, &c.) are got rid of, to at least as great an extent as by the roasting process, by a judicious mixing of the proportions of calcined and 60 raw products, so as to obtain a slag of melted oxide, in more or less quantity upon the liquid bath of metallic copper in the hearth of the furnace. Such non - volatile impurities are naturally collected in this slag, and are 65 skimmed off with it, a suitable flux (such as sand, lime, niter, &c.) being added to the refinery charge when very impure matte is operated on. Although matte of seventy-six to seventy-eight per cent. of copper is preferred, correspondingly good results are obtained from poorer mattes.

The actual cost of practically working this method has been found to be less than half the cost of the ordinary method, as carried 75 out in well conducted works using the old method.

Although we use by preference matte of seventy-six to seventy-eight per cent. of copper and a calcined portion of the same or 80 other matte, our invention applies with correspondingly good results to all matte of from forty-five to eighty per cent of copper.

Having fully described our invention, what we claim, and desire to secure by Letters Pat- 85 ent, is—

The herein described method of producing refined copper from copper matte, consisting in crushing the matte, calcining a proportion of the crushed matte, mixing therewith a 90 suitable portion of uncalcined matte, charging said mixture directly into a refinery furnace and melting the same and finally refining the product in the same furnace on the hearth thereof whereby the material is thus 95 reduced to refined copper by a continuous process in the same furnace, substantially as described.

In testimony whereof we have signed our names to this specification in the presence of 100 two subscribing witnesses.

THOMAS DAVIES NICHOLLS.

CHRISTOPHER JAMES.

Witnesses:

EDWIN GEORGE PROMEROF,

DAVID RICHARD BOWLER.